

June 8, 1965

T. I. JONES

3,188,202

ALUMINUM-PLUTONIUM ALLOYS

Filed April 19, 1961



Figure 1. Al + 5 wt.% Pu Alloy--  
Control  
X 420  
Light phase: Al dendrites  
Dark phase:  $\text{Al}/\text{PuAl}_4$  eutectic



Figure 2. Al + 5 wt.% Pu +  
1 wt.% Ni Alloy  
X 420



Figure 3. Al + 5 wt.% Pu +  
15 wt.% Si Alloy  
X 420



Figure 4. Al + 5 wt.% Pu +  
15 wt.% U Alloy  
X 420



Figure 5. Al + 20 wt.% Pu Alloy  
X 420  
Light phase:  $\text{PuAl}_4$   
Dark phase: eutectic

1

3,188,202

ALUMINUM-PLUTONIUM ALLOYS  
 Thomas Ivor Jones, Deep River, Ontario, Canada, assignor  
 to Atomic Energy of Canada Limited, Ontario, Canada,  
 a corporation

Filed Apr. 19, 1961, Ser. No. 104,183  
 7 Claims. (Cl. 75—122.5)

This invention relates to alloys of aluminum and plutonium, and to methods for their preparation. In particular, the invention includes ternary alloys of aluminum, plutonium and one element selected from the group consisting of uranium, silicon and nickel.

Considerable attention is being devoted to the development of nuclear power reactors which will produce electrical power competitively with the other conventional energy sources. One type of power reactor which is being investigated is water-cooled, in which pressurized water or steam at elevated temperatures (e.g., 250–400° C) is circulated around the fuel rods. The fuel rods are sheathed in a suitable strong, corrosion-resistant alloy (e.g., Zircaloy-2). It is important that, in the event of sheath failure, the coolant system should not become excessively contaminated by the corrosion of the nuclear fuel.

Binary Al-Pu alloys have been found suitable for use as fuel in research reactors operating with low temperature water. The corrosion resistance to high temperature water of Al alloys containing about 13–20 wt. percent Pu and of hyper-eutectic structure, has been found to be good. However, Al alloys containing less than 13 wt. percent Pu and of hypo-eutectic structure, undergo rapid corrosion attack by high temperature water. (T. I. Jones, Second International Conference Plutonium Metallurgy, Grenoble, France, April 1960, IV Session, Paper 1.)

Rod-type fuel elements in water-cooled power reactors, would normally be enriched with less than 13 wt. percent Pu. Al-Pu alloys of up to 13 wt. percent Pu would be of value as fuel elements if they were resistant to corrosion by water at up to about 350° C.

An object of this invention is to prepare a corrosion-resistant aluminum-plutonium alloy of less than 13 wt. percent Pu. Another object is to provide such an alloy which does not absorb neutrons to a significant degree.

I have now found that Al alloys with up to about 8 wt. percent Pu will form ternary alloys with one of the group consisting of nickel, silicon and uranium, which ternary alloys have good corrosion-resistance to high temperature water.

The proportion of Pu in the alloys, giving a suitable enrichment, may range from about 2 to about 8 wt. percent. Four to six wt. percent Pu is presently preferred. The nickel has a relatively large neutron-capture cross-section and its proportion is desirably kept low. From 1 to 2 wt. percent Ni is suitable. The proportions of silicon and uranium fall within the range 13–17 wt. percent, with the total Pu+Si or total Pu+U preferably being within the range 19–21 wt. percent. The hyper-eutectic structure and the absence of any significant free Al phase is ensured at these proportions. Zirconium was found to be unsuitable as a ternary additive since the corrosion resistance to high temperature water was decreased from that of the hypo-eutectic binary alloy.

The alloys are preferably prepared by reducing plutonium dioxide with excess aluminum metal in the presence of cryolite ( $3\text{NaF}\cdot\text{AlF}_3$ ) at about 1100–1200° C., to produce billets of the desired composition. These billets are remelted and the temperature raised to about (a) 775° C. before making the Ni addition, (b) 850° C. before making the Si addition, or (c) 950° C. before making the U addition. The Ni, Si, and U are preferably added in their elemental form. The above preferred tempera-

2

tures of the ternary addition are not critical and may be increased or decreased by about 10° C. to 20° C. or more. However, if the temperatures are much outside these limits non-uniform dispersion, lack of dissolution, presence of dissolved gases, etc. may be the result.

The ternary alloys are then cast into moulds preheated to about 100° C. (e.g., graphite moulds). Other methods may be used for preparing the initial binary alloy such as reducing plutonium trifluoride with excess aluminum or adding Pu metal to Al metal in the melt. (See Runnalls, "Progress in Nuclear Energy," Series V, 2, 98 to 118, Pergamon Press, 1959.)

The following examples will illustrate the invention. Binary alloy of Al and 5 wt. percent Pu was prepared by the reduction of  $\text{PuO}_2$  with excess Al, in the presence of cryolite, at 1150° C. Ternary additions of 1 wt. percent Ni, 15 wt. percent Si and 15 wt. percent U were then made as described above to separate portions of the binary alloy.

Corrosion tests were carried out on the alloys using static de-ionized water at 340° C. This would be a typical temperature of the fuel exterior for a power reactor element cooled by water at 270–280° C. and having a 60–70° C. temperature gradient across Zircaloy-2 sheathing. [Zircaloy-2 is an alloy typically consisting of 1.5% Sn, 0.1% Fe, 0.1% Cr, 0.05% Cr, 0.05% Ni and the balance Zr.] Corrosion test specimens were machined from cast rods, degreased in acetone, etched for one minute in 5% NaOH solution and thoroughly washed in de-ionized water. The time of exposure to the high temperature water was 20 hours. The corrosion test results are summarized in the following Table.

*Corrosion of Al-Pu alloys*

| Alloy                                  | Structure                                                          | Water Temp.<br>°C. | Time<br>(hrs.) | Corro-<br>sive<br>Attack<br>$10^{-3}$ in. |
|----------------------------------------|--------------------------------------------------------------------|--------------------|----------------|-------------------------------------------|
| Al+5 wt. percent Pu                    | Highly refined hypo-eutectic.                                      | 340                | 20             | >125                                      |
| Al+5 wt. percent Pu +1 wt. percent Ni  | Very small equiaxed grains $\alpha$ -Al in a hypo-eutectic matrix. | 340                | 20             | 0.3                                       |
| Al+5 wt. percent Pu +15 wt. percent Si | Highly refined eutectic-like.                                      | 340                | 20             | 0.4                                       |
| Al+5 wt. percent Pu +15 wt. percent U  | do                                                                 | 340                | 20             | 0.6                                       |
| Al+20 wt. percent Pu                   | do                                                                 | 340                | 20             | 0.4                                       |

FIGURES 1 to 5 illustrate the as-cast structures of the alloys listed in the above table.

The Al+5 wt. percent Pu alloy is typical of an alloy having a hypo-eutectic structure with considerable free Al phase being present—as shown in FIGURE 1. This binary alloy is rapidly corroded. The nickel alloy structure includes a hypo-eutectic structure with very small equiaxed grains of  $\alpha$ -Al distributed as shown in FIGURE 2. It will be observed in FIGURES 3–5 that the structures of the 20 wt. percent Pu alloy, the Si alloy and the U alloy, are all quite similar being highly refined and hyper-eutectic. The corrosion resistance of the three ternary alloys is similar to that of the 20 wt. percent Pu alloy.

The corrosion resistance of the ternary alloys is significantly improved relative to the 5 wt. percent plutonium binary alloy—such that the ternary alloys are suitable from a corrosion standpoint for fuel applications using high temperature water coolant.

The above examples are not intended to be limiting. The proportions may be varied as indicated above. Other methods of preparing the initial binary Al-Pu alloy may be used. The uranium in the example was the naturally-occurring mixture of isotopes, but other isotope mixtures may be used. In the above illustrative alloys, super-purity

aluminum was used. Spectrographic analyses of the ternary alloys revealed the following impurities:

Na ..... weight percent <0.03  
 B, Cr, Fe, K, Pb, Ca, Ti, Zn ..... <0.02

However, it is not necessary to use such super-purity aluminum.

I claim:

1. An alloy consisting of from 2 to 8 wt. percent plutonium, uranium from 13 to 17 wt. percent, and the balance aluminum.
  2. The alloy of claim 1 wherein the plutonium is present in from 4 to 6 wt. percent.
  3. The alloy of claim 1 wherein the total plutonium plus uranium concentration is from 19 to 21 wt. percent.
  4. An alloy consisting of about 5 wt. percent plutonium, about 1 wt. percent nickel, and the balance aluminum.
  5. An alloy consisting of about 5 wt. percent plutonium, about 15 wt. percent uranium, and the balance aluminum.
  6. An alloy consisting of from 2 to 8 wt. percent plutonium,

tonium, nickel in from 1 to 2 wt. percent, and the balance aluminum.

7. The alloy of claim 6 wherein the plutonium is present in from 4 to 6 wt. percent.

### References Cited by the Examiner

UNITED STATES PATENTS

|           |       |                  |          |
|-----------|-------|------------------|----------|
| 2,885,283 | 5/59  | Schonfeld et al. | 75—122.5 |
| 2,919,186 | 12/59 | Colbeck          | 75—122.7 |
| 2,929,706 | 3/60  | Cramer et al.    | 75—122.7 |
| 2,934,424 | 4/60  | McKenzie         | 75—84.1  |
| 2,992,915 | 7/61  | Nelson           | 75—84.1  |

#### OTHER REFERENCES

- 15 AEC Report ANL-5430, July 1955, pp. 22, 23, 25, 27-  
29, 31, and 33.

Nuclear Science Abstracts, vol. 14, pp. 2317 and 2318. Abstracts Nos. 18109 and 18110, Sept.-Oct. 1960.

Nuclear Science Abstracts, vol. 13, pp. 24 and 25.  
20 Abstracts Nos. 191, 192, 194, and 197, Jan.-Feb. 1959.

CARL D. QUARFORTH, *Primary Examiner.*

OSCAR R. VERTIZ, *Examiner.*